

1

3,406,107

**NON-CYANIDE SILVER PLATING BATH**  
Kurt R. Grebe, Beacon, and John V. Powers, Shenorock,  
N.Y., assignors to International Business Machines Cor-  
poration, Armonk, N.Y., a corporation of New York  
No Drawing. Filed Dec. 7, 1964, Ser. No. 416,594  
2 Claims. (Cl. 204—46)

**ABSTRACT OF THE DISCLOSURE**

A non-cyanide silver plating bath is described. The bath is composed of ammonium phosphate, sodium phosphate and silver nitrate. Silver films deposited from the above bath are mirror bright, ductile and have excellent adhesive properties with respect to the substrates upon which the films are deposited.

This invention relates to the electrodeposition of silver, and more particularly to the improved electrodeposits of silver employing soluble or insoluble anodes.

It is very desirable in the art of electroplating silver to avoid the use of cyanide in such baths. Although cyanide silver plating baths are commercially feasible, they have the defect of being poisonous and must be operated under highly controlled conditions. Attempts have been made to obtain non-cyanide silver plating baths to avoid employing a dangerous or noxious substance in such baths, but such non-cyanide silver plating baths have been inefficient to the point of making them of questionable value in a commercial operation.

Consequently, it is an object of this invention to provide a non-cyanide silver plating bath that is economically feasible in its operation and competitive with cyanide silver plating baths.

It is yet another object to obtain a non-cyanide silver plating bath which has high speed in its operation, produces a mirror bright silver deposit, is extremely ductile and has excellent adhesive properties with respect to a substrate on which said silver is deposited.

It is a further object to provide a non-cyanide silver plating bath that is exceedingly stable.

A further object is to obtain a non-cyanide plating bath having good "throwing" power and whose cathode efficiency is approximately 100%.

The foregoing and other objects, features and advantages of the invention will be apparent from the following more particular description of a preferred embodiment of the invention.

The new bath comprises ammonium phosphate, sodium phosphate, silver nitrate, all dissolved in water. A representative bath would comprise 20 grams of ammonium phosphate, 100 grams of sodium phosphate, 10 grams of silver nitrate and sufficient water to make 1 liter of the solution. The bath is maintained at a temperature between 25°—95° C., should have a pH of 8.5 or higher and the current density of the electrodes in the bath should be 15—45 ma./sq. inch.

During the passage of current between the cathode and the anode of the electroplating bath, wherein said anode could either be soluble or insoluble, the ammonium phosphate is a source of ammonium ions, the latter serving to complex the silver. Although the representative

2

solution shows a ratio of ammonium phosphate to silver nitrate of 2:1, the ratio of ammonium phosphate to silver nitrate can be made as high as 10:1 without interfering with the efficiency of the non-cyanide silver plating bath. Moreover, in the example given, the ratio of sodium phosphate to silver nitrate is 10:1, such ratio can be altered to be as high as 40 or 50:1 without interfering with the operation of the plating bath. Since the sodium phosphate is employed to add to the conductivity of the electroplating solution there is a wide variation in the amount of sodium phosphate permitted. Although a temperature range of 25°—95° C. is suggested, optimum depositions are obtained at about 35° C.

The non-cyanide silver plating solution described above has been found to be exceedingly stable wherein long shelf storage has not appreciably altered the brightness, nor ductility nor adhesive qualities of the bath. The silver deposits have been found to be in an unstressed condition and the extremely good throwing power of such plating solution has made it highly desirable for plating irregularly shaped objects.

According to this invention there is provided a non-cyanide silver plating bath having the following composition:

|    |                    |        |         |
|----|--------------------|--------|---------|
| 25 | Ammonium phosphate | g./l.  | 20—100  |
|    | Sodium phosphate   | g./l.  | 100—500 |
|    | Silver nitrate     | g./l.  | 10—50   |
|    | Water              | liters | 1       |
| 30 | pH                 |        | >8.5    |

While the invention has been particularly described with reference to a preferred embodiment thereof, it will be understood by those skilled in the art that various changes in form and details may be made therein without departing from the spirit and scope of the invention.

What is claimed is:

1. A non-cyanide bath for electroplating silver consisting of essentially of 20—100 g./l. of ammonium phosphate, from 100—500 g./l. of sodium phosphate, from 10—50 g./l. of silver nitrate, the balance water, said bath having a pH of 8.5 or higher.

2. A low temperature non-cyanide bath for electroplating silver consisting of:

|    |                    |        |      |
|----|--------------------|--------|------|
| 45 | Ammonium phosphate | grams  | 20   |
|    | Sodium phosphate   | do     | 100  |
|    | Silver nitrate     | do     | 10   |
|    | Water              | liters | ≤1   |
| 50 | pH                 |        | ≥8.5 |

**References Cited**

**UNITED STATES PATENTS**

|         |           |        |           |        |
|---------|-----------|--------|-----------|--------|
| 744,170 | 11/1903   | Darlay | 204—46 X  |        |
| 923,864 | 6/1909    | Levy   | 204—46 XR |        |
| 55      | 2,504,272 | 4/1950 | McCoy     | 204—46 |

**FOREIGN PATENTS**

|         |         |                |
|---------|---------|----------------|
| 939,007 | 10/1963 | Great Britain. |
|---------|---------|----------------|

**OTHER REFERENCES**

American Chemical Journal, p. 335, vol. 12, 1890.

HOWARD S. WILLIAMS, *Primary Examiner.*

G. KAPLAN, *Assistant Examiner.*